

## UNITED STATES PATENT OFFICE

EDOUARD M. KRATZ, OF CHICAGO, ILLINOIS, ASSIGNOR TO MARSENE PRODUCTS CO.,  
A CORPORATION OF ILLINOIS

## TRANSPARENT SHEET MATERIAL

No Drawing.

Application filed August 15, 1927. Serial No. 213,225.

This invention relates to transparent sheet material adapted for use as wrapping for candy boxes, bonbons, flowers and the like.

In my copending application entitled, "Transparent sheets and the process of manufacture", Serial No. 10,962, filed February 21, 1925, I have disclosed a method of making transparent sheet material from gelatine and sulphonated castor oil. I have now found that if a glycol, such as ethylene glycol, di-ethylene glycol, or the ethyl ether of di-ethylene glycol is used wholly or partly in place of sulphonated castor oil, a very satisfactory, relatively non-hygroscopic sheet is obtained. I have further found that a small amount of sulphonated castor oil or other grease dispersing agent is practically essential for the formation of a satisfactory sheet.

This invention has, therefore, for one of its objects to provide an improved composition for forming relatively non-hygroscopic transparent sheet material from gelatine and a glycol, together with a suitable grease dispersing agent.

Other and further important objects of this invention will become apparent from the disclosures in the following description and appended claims, which set forth a preferred form of my invention.

The proportion of glycol to gelatine may be varied over a considerable range, depending upon the qualities desired in the sheet. Gelatine sheets, as is well-known, are extremely hygroscopic and fragile, and are subject to great physical change with varying atmospheric conditions. Glycol, including certain of its homologs, serves as a softening agent for the gelatine and renders it substantially non-hygroscopic and pliable.

Ordinarily, the percentage of glycol in the finished sheet material will range between limits of 5 and 60%. Below 5% the resulting sheets would be too hard and brittle, and above 60% they would be too soft and lack coherence. A more satisfactory range would be from 15 to 40% of glycol and the balance largely gelatine. A part of the glycol content may be replaced by sulphonated castor oil, and, in fact, it is preferable to add a small quantity of sulphonated castor oil in order

to disperse the grease and fats normally present in even the highest grades of gelatine. In place of sulphonated castor oil, a small quantity of ox-gall may be used. If desired, a hardening or tanning agent, such as formaldehyde or chrome salts, may be added to increase the insolubility of the sheets.

I prefer to use a composition containing on a dry basis about 25% of an ethylene glycol mixture, 70% of gelatine and about 5% of 40% formaldehyde. The ethylene glycol mixture preferably comprises 60% ethylene glycol, 30% glycerine and 10% sulphonated castor oil (8% sulphonated). Ordinarily, glycerine is very objectionable on account of its hygroscopic properties, but in combination with glycol, it appears to lose these properties. In order to obtain a clear white transparent sheet, it is usually advisable to add a small quantity of a blue dyestuff, such as alizarine sapphirol. For obtaining colored sheets, larger quantities of dyes may be used the same as in dyeing gelatine sheets.

In my process of manufacture, the glue is first soaked in four times its weight of cold water for at least six hours and then melted at 115° F. The ethylene glycol mixture is diluted and then added to the gelatine solution with agitation, the temperature being maintained between 100 and 120° F. To counteract the yellow cast in the natural sheet, about 0.5% of alizarine sapphirol by weight of the dry gelatine composition, is added to the solution. A small quantity of a tanning agent may be added if desired. The mass is then diluted with soft water at 120° F. to the viscosity required to give the desired sheet. The sheet is preferably formed on an endless belt, such as described in my application entitled, "Surface for forming transparent paper", Serial No. 11,335, filed February 24, 1925. The belt containing a film of the gelatine composition solution, is passed through a chill box to set the sheet and finally dried by hanging in festoons in a suitable drying rack. The sheet material so formed may be readily stripped from the belt and cut into transparent, self-sustaining sheets, that are

relatively non-hygroscopic and unaffected by climatic conditions.

The gelatine used should be glue of the highest quality, free from preservatives, especially zinc sulphate. The sulphonated oil, if any is used, is preferably castor oil that has been sulphonated so as to contain between 4 and 10% by weight of the sulphonic acid radical ( $\text{HSO}_3$ ). The sulphonated oil should be thoroughly washed and neutralized with sodium or potassium hydroxide. An ammonia-neutralized oil is not satisfactory, as it produces a milky sheet. In place of ethylene glycol, di-ethylene glycol or the mono ethyl ether of di-ethylene glycol may be substituted.

I am aware that many changes may be made and numerous details of the process may be varied through a wide range without departing from the principles of this invention and I, therefore, do not purpose limiting the patent granted hereon, otherwise than necessitated by the prior art.

I claim as my invention:

1. Transparent sheet material, comprising gelatine, a water soluble paraffin glycol, and a grease dispersing agent.
2. Transparent sheet material, comprising gelatine, ethylene glycol, and a grease dispersing agent.
3. Transparent sheet material, comprising 40 to 95% of gelatine, 60 to 5% of ethylene glycol, and a grease dispersing agent.
4. Transparent sheet material, comprising about 25% of a mixture containing ethylene glycol, glycerine and sulphonated castor oil, 70% of gelatine and 5% of a tanning agent.
5. A self sustaining transparent sheet, comprised largely of gelatine and ethylene glycol, said sheet being relatively non-hygroscopic and flexible.
6. A self sustaining transparent sheet, comprised of 60 to 85% of gelatine and 40 to 15% of an ethylene glycol mixture, containing sulphonated castor oil, glycerine and a tanning agent.
7. A self sustaining transparent sheet, comprised largely of gelatine and ethylene glycol, and relatively smaller quantities of sulphonated castor oil and a tanning agent.

In testimony whereof I have hereunto subscribed my name.

EDOUARD M. KRATZ.